# EUROPEAN PATENT SPECIFICATION

(11) **EP 0 826 222 B1**
(45) Date of publication and mention of the grant of the patent: **27.12.2000**
(21) Application number: 96912148.2
(22) Date of filing: 03.05.1996
(51) Int. Cl.: H01B 13/32

(54) **METHOD OF BLOCKING A CABLE OR BUNDLE OF CONDUCTORS**
VERFAHREN ZUM ABDICHTEN VON EINEM KABEL ODER LEITERBÜNDEL
PROCEDE DE BLOCAGE DE CABLE OU D'UN FAISCEAU DE CONDUCTEURS

(30) Priority: 18.05.1995 GB 9510031; 05.12.1995 GB 9524885
(43) Date of publication of application: 04.03.1998
(73) Proprietor: RAYCHEM LIMITED, Dorcan, Swindon, Wiltshire SN3 5HH (GB)
(72) Inventor: CROFTS, David, Cirencester Gloucestershire GL7 6DT (GB)
(74) Representative: Jay, Anthony William
(86) International application number: GB9601062
(87) International publication number: WO9636976

(56) References cited:
- EP-A- 0 249 510
- WO-A-94/24837

## Description

This invention relates to a method of blocking a cable or bundle of conductors.

Blocking to prevent fluids from flowing along a cable or wire bundle is known, for example from US-A-4972042 (RK310), wherein a body of hot-melt adhesive is placed in contact with the (usually insulated) conductors and a heat-shrinkable sleeve is shrunk around the portion of the cable or bundle carrying the adhesive. The heat applied to shrink the sleeve, usually by means of a hot air gun or a flame torch, causes the adhesive to melt and flow between and around the conductors, assisted by the shrinking action of the sleeve, thus blocking the cable or bundle. These known blocking procedures are subject to the limitations that the adhesive must be able to melt and flow at relatively low temperatures, often less than 100°C, which can be achieved inside the sleeve without overheating and damaging it. This can undesirably limit the temperatures which can be tolerated by the blocked cable or bundle in subsequent service.

An alternative cable blocking system is described in WO-A-94/24837 (MP1474), wherein particles of ferromagnetic material are incorporated in hot melt blocking adhesive, the particles being shaped to couple inductively with an alternating magnetic field to which the cable carrying the adhesive is subjected. The resulting inductive heating of the specially-shaped ferromagnetic particles causes the adhesive to melt and flow to block the cable. A heat-shrinkable sleeve is also provided with the ferromagnetic particles to heat it to its shrinkage temperature on exposure to the magnetic field. This system alleviates the aforementioned limitations of external heating.

The present invention also avoids external heating while ingeniously reducing or eliminating the need for the specially-shaped ferromagnetic particles, which may be expensive or otherwise undesirable to use in some circumstances.

The invention accordingly provides, in its broadest aspect, a method of blocking a cable or bundle of inductively-heatable, preferably metallic, conductors, comprising (a) applying to a portion of the cable or bundle to be blocked a body of heat-flowable blocking material; (b) optionally applying around at least the portion of the cable or bundle to be blocked a cover; wherein the blocking material is substantially electrically non-conductive and substantially non-magnetic and therefore substantially non-inductively-heatable, and the cover is inductively-heatable or substantially electrically non-conductive and substantially non-magnetic and therefore substantially non-inductively-heatable or absent and (c) subjecting the cable or bundle to an alternating magnetic field which couples inductively (I) with the said conductors and (II) with the inductively-heatable cover when present, thereby inductively heating the conductors to a temperature which causes the blocking material to flow and block the cable or bundle.

The invention is based on the surprising discovery that sufficient heat can be inductively generated in the conductors, in the substantial absence of induction-heatable additives in the blocking material, to melt and flow the blocking material to achieve a satisfactory block. The invention has the advantage of being equally applicable when a cover is provided around at least the portion of the cable or bundle to be blocked. Such a cover may be an article which is elastomeric and is arranged to compress the said portion on the cable or bundle at least before and during the flowing of the blocking material.

It is even more surprising that the cover may be a heat-shrinkable article which is caused to shrink around the said portion of the cable or bundle. This novel use of heat generated by the conductors inside the cable or bundle advantageously enables blocking materials of higher melting or softening temperatures to be used without damage to the heat-shrinkable cover. Alternatively, the heat-shrinkable article might carry induction-heatable additives within itself or in an internal lining of an adhesive or other material, so that only the blocking material relies on the heat generated in the conductor.

The melting or softening point of the blocking material, and the threshold shrinkage temperature of the heat-shrinkable cover, if present, will normally be selected to suit temperatures which can be generated by the induction heating of the conductors without damage to any electrical insulation materials carried by the conductors. For example car harness with up to 100 wires made of PVC-insulated wires of diameters 0.25 to 6 mm² with a temperature rating of 105°C (T2 Rating) can be blocked within 3 minutes using an adhesive with a softening temperature of 85°C and a flow temperature of 110°C with a heat-shrinkable sleeve of recovery temperature below 100°C, and using an induction generator operating at a frequency between 0.2 and 1 Mhz with 2.5 kW power. Lower-temperature-rated (i.e. T1 =70°C) PVC requires the use of hot-melt adhesives with softening points of 50 - 60°C and flow temperatures of 80 - 90°C with heat-shrinkable tubing of recovery temperatures less than 90°C.

As an alternative blocking adhesive for wire with low insulation softening points in the range of 50 - 60°C, the melt adhesive can be replaced with a mastic material such as polyisobutylene. During installation the heat from the wires softens the mastic and increases its flow. Under these circumstances either a heat-shrink sleeve or a rubber sleeve can be used to consolidate the block.

This invention is especially applicable to conductors composed of fine metal filaments whose geometry lends itself to inductive coupling with the applied magnetic field, for example copper wire consisting of many individual strands typically 75 to 150 micro-metres in diameter. These are roved together to make the wire and typically from 7 to 50 strands can be used depending on the final cross sectional area of the wire. The normal material is copper and it may be plated with either nickel, tin or silver. However, other conductor materials can be used such as nickel or aluminium.

Any suitable blocking material may be used which will flow at the temperatures generated by the conductors and will solidify sufficiently to block the cable in subsequent service. Preferred hot melt adhesives are those described in the aforementioned US-A-4972042.

The heat-shrinkable cover will preferably be as described in US-A-4972042 or in WO-A-94/24837.

When an elastomeric cover is used, this may be made of, for example, EPDM rubber, polychloroprene rubber, polyester rubber, or natural rubber. The size and shape of the cover are not critical, provided that it squeezes the assembly sufficiently to confine the following blocking material in position to form an adequate block in the cable or bundle.

Specific examples of this aspect of the present invention will now be described in more detail by way of further illustration.

### EXAMPLE 1

A wire bundle consisting of 60 1.5mm² copper conductors of 100 micron diameter strands with a 0.5mm jacket of PVC insulation rated to T2 (105°C) was blocked using Rayblock 85® Polyamide hot melt adhesive applied in the form of 4, 5 channel comb profiles. The wires were fitted into each channel of the comb with a maximum of three wires per channel. The outer heat shrink tubing was a 40mm length of TAT-125® heat shrink tubing 25mm in diameter. A 250kHz induction heater was used to generate a field within a 5 turn 50mm diameter helical coil. The coil was operated at 150 amps giving a filed strength of 750 ampere turns and the cable harness was blocked in 60 seconds, the maximum temperature reached in the bundle was 130°C.

### EXAMPLE 2

A bundle as described in Example 1 except that a 40mm sleeve of 15mm diameter chloroprene rubber of 60IRHD hardness was used instead of the heat shrink sleeving. Under the same conditions as that example the sample was blocked in 45 seconds.

### EXAMPLE 3

A bundle as described in Example 1 was blocked using a poly iso butylene mastic (3M's EMB-45R®) with a chloroprene rubber sleeve as described in Example 2. The sample was heated in the induction heater for 60 seconds during which time the mastic flowed from under the elastomeric tubing and completed the sealing process.

### EXAMPLE 4

### A bundle as described by Example 1 except the insulation on the wire was

Raychem Type 62® polyester wire with a temperature rating of T3 (125°) was used with polyamide adhesive combs Rayblock 105®. The heat shrink sleeve was Raychem ATUM 24/8 (Trade Mark) and the bundle was heated for 90 seconds to seal with a maximum temperature of 160°C being recorded in the bundle.

When the substantially non-inductively heatable cover is heat-shrinkable, it will preferably shrink at temperatures which it encounters as a result of the inductive heating and/or the resultant flowing of the blocking material.

When the cover is elastomeric, it will preferably be arranged to compress the portion of the cable or bundle to be blocked at least before and during the flowing of the blocking material.

For non-inductively-heatable blocking materials in all aspects of the present invention, it may be desirable in some cases to use materials which are curable so that their viscosity increases after flowing and blocking the cable or bundle, thus reinforcing the blocking effect and reducing the risk of the block becoming ineffective due to later temperature variations. Preferred curable blocking materials may be selected from those comprising interleaved sheets containing respectively the separate reactive components of a curing system, which are described in WO-A-9527764 (B247).

## Claims

1. A method of blocking a cable or bundle of inductively-heatable, preferably metallic, conductors, comprising
a applying to a portion of the cable or bundle to be blocked a body of heat-flowable blocking material;
b optionally applying around at least the portion of the cable or bundle to be blocked a cover; wherein the blocking material is substantially electrically non-conductive and substantially non-magnetic and therefore substantially non-inductively-heatable, and the cover is inductively-heatable or substantially electrically non-conductive and substantially non-magnetic and therefore substantially non-inductively-heatable or absent and
c subjecting the cable or bundle to an alternating magnetic field which couples inductively (I) with the said conductors and (II) with the inductively-heatable cover when present, thereby inductively heating the conductors to a temperature which causes the blocking material to flow and block the cable or bundle.

2. A method according to claim 1, wherein the cover is a heat-shrinkable article which is caused to shrink around the said portion of the cable or bundle.

3. A method according to claim 2, wherein the heat-shrinkable article shrinks at temperatures which it encounters as a result of (i) the inductive heating of the conductors, and/or (ii) the resulting flowing of the blocking material.

4. A method according to claim 1, wherein the cover is elastomeric and is arranged to compress the said portion of the cable or bundle at least before and during the flowing of the blocking material.

## Patentansprüche

1. Verfahren zum Blockieren eines Kabels oder eines Bündels aus induktiv erwärmbaren, bevorzugt metallischen Leitern, wobei das Verfahren die folgenden Schritte aufweist:
(a) Aufbringen eines Körpers aus unter eines Wärmeeinwirkung fließfähigem Blockiermaterial auf einen Bereich des zu blockierenden Kabels oder Bündels;
(b) fakultatives Aufbringen einer Abdeckung zumindest um den zu blockierenden Bereich des Kabels oder Bündels herum; wobei das Blockiermaterial im wesentlichen elektrisch nicht leitfähig und im wesentlichen nicht magnetisch und somit im wesentlichen nicht induktiv erwärmbar ist und die Abdeckung induktiv erwärmbar oder im wesentlichen elektrisch nicht leitfähig und im wesentlichen nicht magnetisch und somit im wesentlichen nicht induktiv erwärmbar oder abwesend ist, und
(c) Anlegen eines Wechselmagnetfelds an das Kabel oder Bündel, wobei das Wechselmagnetfeld induktiv (I) mit den Leitern und (II) mit der induktiv erwärmbaren Abdeckung, wenn vorhanden, gekoppelt wird, so daß die Leiter induktiv auf eine Temperatur erwärmt werden, die das Blockiermaterial zum Fließen und zum Blockieren des Kabels oder Bündels veranlaßt.

2. Verfahren nach Anspruch 1,
wobei die Abdeckung ein durch Wärme schrumpfbarer Gegenstand ist, der veranlaßt wird, um den Bereich des Kabels oder des Bündels herum zu schrumpfen.

3. Verfahren nach Anspruch 2,
wobei der durch Wärme schrumpfbare Gegenstand bei Temperaturen schrumpft, die er erfährt als Ergebnis (i) des induktiven Erwärmens der Leiter und/oder (ii) des resultierenden Fließens des Blockiermaterials.

4. Verfahren nach Anspruch 1,
wobei die Abdeckung elastomer und so angeordnet ist, daß sie den Bereich des Kabels oder des Bündels zumindest vor dem Fließen oder während des Fließens des Blockiermaterials zusammendrückt.

## Revendications

1. Procédé de blocage d'un câble ou d'un faisceau de conducteurs, avantageusement métalliques, pouvant être chauffé par induction, comprenant
(a) l'application à une portion du câble ou du faisceau devant être bloquée d'une masse de matière de blocage pouvant s'écouler sous l'effet de la chaleur ;
(b) l'application facultative d'une enveloppe autour au moins de la portion du câble ou du faisceau devant être bloquée ; dans lequel la matière de blocage est substantiellement électriquement non conductrice et substantiellement non magnétique et, par conséquent, ne peut donc substantiellement pas être chauffée par induction, et l'enveloppe peut être chauffée par induction ou est substantiellement électriquement non conductrice et substantiellement non magnétique et, par conséquent, ne peut substantiellement pas être chauffée par induction ou est absente, et
(c) la soumission du câble ou du faisceau à un champ magnétique alternatif qui réalise un couplage inductif (I) avec lesdits conducteurs et (II) avec l'enveloppe pouvant être chauffée par induction, lorsqu'elle est présente, chauffant ainsi par induction les conducteurs à une température qui amène la matière de blocage à s'écouler et à bloquer le câble ou le faisceau.

2. Procédé selon la revendication 1, dans lequel l'enveloppe est un article thermorétractable qui est amené à se rétracter autour de ladite portion du câble ou du faisceau.

3. Procédé selon la revendication 2, dans lequel l'article thermorétractable se rétracte à des températures qu'il rencontre par suite (i) du chauffage par induction des conducteurs, et/ou (ii) de l'écoulement résultant de la matière de blocage.

4. Procédé selon la revendication 1, dans lequel l'enveloppe est élastomérique et est agencée de façon à comprimer ladite portion du câble ou du faisceau au moins avant et pendant l'écoulement de la matière de blocage.
